

G. J. BOHLMAN.

METHOD OF FORMING PAPER ARTICLES.

APPLICATION FILED FEB. 19, 1915.

1,175,406.

Patented Mar. 14, 1916.



*Fig. 1.*



*Fig. 2.*



Witnesses:

H. B. Davis.  
R. Connell.

*Fig. 3.*



*Fig. 4.*

Inventor:  
George J. Bohlman  
by Mayo & Hannigan  
Attest.

# UNITED STATES PATENT OFFICE.

GEORGE J. BOHLMAN, OF MEDFORD, MASSACHUSETTS, ASSIGNOR TO AMERICAN WATER SUPPLY CO., OF BOSTON, MASSACHUSETTS, A CORPORATION OF MAINE.

## METHOD OF FORMING PAPER ARTICLES.

1,175,406.

Specification of Letters Patent. Patented Mar. 14, 1916.

Original application filed November 2, 1914, Serial No. 869,763. Divided and this application filed February 19, 1915. Serial No. 9,261.

To all whom it may concern:

Be it known that I, GEORGE J. BOHLMAN, a citizen of the United States, residing at Medford, in the county of Middlesex and 5 State of Massachusetts, have invented an Improvement in the Methods of Forming Paper Articles, of which the following is a specification.

This invention relates to the manufacture 10 of articles of paper, such for instance, as paper drinking cups, and is a division of my application #869,763, filed November 2, 1914. The article herein illustrated is the paper drinking cup of my said application. 15 The characteristic novel feature of said cup is a rolled edge at either or both ends of its body. The cup, together with its rolled edge, is rendered substantially waterproof by treatment with paraffin wax, and the 20 present invention has for its object, a novel method of manufacturing cups which is adaptable to other articles composed of paper, said method being a simple one and requiring but little paraffin.

25 In carrying out my invention, the cup body or other article is formed in any usual or suitable manner, and in case of a cup, its bottom piece is arranged therein, and while said cup-body is on the form on which it is made, or on a similar form, the paraffin is applied to it in the form of a liquid spray at a high temperature, which is caused to spread over its entire outer surface, and, as a result, the paper becomes saturated as well 30 as coated with a layer of uniform thickness, and is, therefore, in temper, and while in such condition, it can be easily bent and slightly stretched without breaking. While 35 said body is in temper, one or both of its end-portions are subjected to a suitable bending or edge-rolling device, by which they are rolled over, thereby to produce a rolled edge at either or both ends, and then 40 said body is allowed to cool and the paraffin 45 to set or congeal, whereupon the paper becomes quite stiff and its rolled edge becomes permanently set.

Figure 1, is a side elevation and partial longitudinal vertical section of a paper 50 drinking cup having both of its ends rolled by the method herein involved. Fig. 2, is a similar view of a paper drinking cup, its up-

per edge only being rolled. Fig. 3, is a side elevation of a paper cup before its edges are rolled, and illustrating the sprays or jets of 55 paraffin wax which are being directed upon the cup-body, and the molds or forms which serve as bending-devices. Fig. 4, is a similar view showing the cup-body with its end- 60 portions rolled over.

10 represents a paper cup-body, and 12 a bottom-closure therefor, both of which may be of any well-known or suitable construction. After the body is produced, it is placed on a form 15, or while reposing on 65 the form on which it is made, a spray or jet of melted paraffin wax, indicated at 16, is directed upon it, which is extended over its entire surface, and which acts to coat the body but more particularly to saturate the 70 paper, so that it is in good temper, and may be easily bent without breaking. While the cup-body is in temper, its ends are rolled over by a suitable stretching and bending-device, such for instance, as represented in 75 Fig. 3, wherein a plate 20 is arranged at the bottom of the form 15 having a shallow groove 21, semicircular in cross-section, adapted to receive the lower end of the cup-body, and by a slight downward pressure 80 upon said body its end-portion or edge is caused to follow the curved wall of said groove and thereby to stretch and bend outwardly, upwardly and then inwardly, sub- 85 substantially completing a circle, although the distance said bend is continued may vary more or less. Also, a similarly grooved plate 30, is or may be arranged above the form, the groove 31 of which receives the upper end-portion of the cup-body, as said 90 plate and form are moved one toward the other, with the result that said end-portion is similarly bent. After the bend or bends are formed the cup-body is allowed to cool 95 whereupon the paraffin congeals, and the pa- 100 per is caused to remain in the position in which it is bent, becoming permanently set. The rolled edge or edges thus formed are quite stiff, and are coated with a layer of uniform thickness on the underside with

wax, and although of small diameter they are sufficiently rigid to prevent the edge being broken by any pressure or strain upon them to which they are ordinarily subjected,

and provide smooth rounded lip-engaging portions which will not have a tendency to cut the lip.

I claim:—

- 5 1. The method herein described of forming paper articles, which consists in making the article of paper, then simultaneously saturating and heating the paper with melted paraffin wax, and while the paper is thus saturated, and in a temper, bending it into the desired form and then allowing the article to cool, whereupon the paraffin congeals and the article thus formed becomes permanently set.
- 10 15 2. The method herein described of forming paper articles, which consists in making the article of paper, then simultaneously saturating and heating the paper with melted paraffin wax, and while the paper is thus saturated, and in a temper, stretching and bending it into the desired form and then allowing the article to cool, whereupon the paraffin congeals and the article thus formed becomes permanently set.
- 20 25 3. The method herein described of forming rolled edges on cup-bodies, which consists in forming the cup-body, subsequently applying to the outside of said body, melted

paraffin wax, which saturates the paper, composing the cup-body, throughout its entire length, and while the paper is thus saturated and in temper, bending the end-portion of the body to form a rolled edge and then allowing said body to cool whereupon the paraffin congeals and the rolled edge becomes permanently set.

4. The method herein described of forming rolled edges on cup-bodies, which consists in forming the cup-body, subsequently applying to the outside of said body, melted paraffin wax, which saturates and simultaneously heats the paper, composing the cup-body, throughout its entire length, and while the paper is thus saturated and in temper, stretching and bending the end-portion of the body to form a rolled edge and then allowing said body to cool, whereupon the paraffin congeals and the rolled edge becomes permanently set.

In testimony whereof, I have signed my name to this specification in the presence of two subscribing witnesses.

GEORGE J. BOHLMAN.

Witnesses:

KATHERINE G. McNAMARA,  
AMOS L. TAYLOR.